

Oct. 2, 1951

H. J. READING

2,569,577

## METHOD OF AND APPARATUS FOR ELECTROPLATING

Filed May 9, 1947

2 Sheets-Sheet 1



**INVENTOR.**  
**HARRY J. READING.**

BY  
*James J. Shanley*  
ATTORNEY

Oct. 2, 1951

H. J. READING

2,569,577

METHOD OF AND APPARATUS FOR ELECTROPLATING

Filed May 9, 1947

2 Sheets-Sheet 2



INVENTOR.  
HARRY J. READING.

BY

*James J. Cleary*  
ATTORNEY

## UNITED STATES PATENT OFFICE

2,569,577

METHOD OF AND APPARATUS FOR  
ELECTROPLATING

Harry J. Reading, Steubenville, Ohio, assignor to  
National Steel Corporation, a corporation of  
Delaware

Application May 9, 1947, Serial No. 747,006

11 Claims. (Cl. 204—28)

1

The present invention relates to improvements in a method of and apparatus for electrodepositioning a protective metal coating onto at least one surface of a continuously moving strip of conductive base metal and more particularly relates to improvements in circulating and discharging replenishing solution into an electroplating cell of the type used for depositing progressively a metal coating on the bottom surface of a horizontally and continuously moving metal strip.

The present invention will be described more particularly in connection with electrolytically coating ferrous metal strip with tin, although it is to be understood that its principles may be followed in electrolytically depositing other protective metals on strips of other conductive materials.

This invention is concerned with the electroplating process in which the strip is passed continuously across one cell, or a series of cells, each containing a tin anode. The strip is passed across each cell above the anode and substantially at the level of the surface of the electrolyte bath contained in the cell so that only the bottom surface of the strip is plated. When it is desirable to coat the opposite surface, the direction of the strip travel is reversed to position the other surface downwardly and the strip is then passed across a second series of plating cells in which the other surface is similarly coated. The strip passes across the plating cell at a speed of 500 feet, or more, per minute. Speeds of 1,000 to 1,500 feet per minute are used in many present commercial installations. The electrolyte solution in each cell flows out of the cell and usually flows across the side walls of the cell that are located at such a level as to maintain the quiescent level of the bath at or slightly above the level of the bottom of the strip. Electrolyte solution is continuously fed into the cell so as to replenish the bath and maintain the proper concentration of tin salts in the bath.

In continuously electroplating ferrous metal strip with tin commercially, a persistent source of trouble has been the formation of heavier deposits of tin along the edges of the strip as a result of higher current density. Another trouble encountered has been the deposition of electrolyte salts along the edges of the upper surface. Dams have been placed across the exit end of the cell so that all, or substantially all, of the electroplating solution flows out of the cell across the top of the side wall at the entry end of the cell tray. This dam stops the flow of solution in the direction of

5 strip travel so that at the exit end, the level of the solution builds up above the surface of the strip whereby the solution flows back along the upper surface and aids in wetting the surface and preventing the deposition of salts on the upper surface. The anodes in the cells have been carefully arranged in an effort to reduce the increased current density and resulting thickness of tin along the edges of the strip. Such efforts have not met with entire success for the tin coating has continued to be thinner along the middle portion of the strip than along the edge portions. This has increased the amount of coated strip that has had to be scrapped and has further increased the cost in that a heavier coating of tin than necessary must be deposited along the edge portions to provide the required amount of tin on the middle portion.

Accordingly, one of the primary objects of the present invention is to prevent or reduce the increased thickness of the tin coating along the edges of electroplated strip.

Another object is continuously to electroplate strip with a uniform coating of protective metal that has substantially the same thickness along the middle portion as along the edge portions.

A further object of the present invention is to provide an improved method of and apparatus for continuously electroplating ferrous metal strip with a uniform coating of tin on the bottom surface and without the deposition of electrolyte salts on the upper surface.

I have discovered that the reduced thickness of the tin coating along the mid-portion of the strip is not entirely a result of reduced current density along this portion, but that the manner in which the electrolyte solution is discharged into the electroplating cell materially affects the thickness of the coating on the bottom surface. This is somewhat surprising as it has been considered heretofore that it was the distribution of the current density which affects the thickness of the coating and that it was only necessary to maintain absolute uniformity of current density to produce a coating of the same thickness along all zones. Although some consideration has been given to the way in which the replenishing electrolyte solution was discharged into the cell, the aim heretofore has been to add the solution so that all portions of the bath would contain substantially the same amount of electrolyte salts. It has been assumed that if the bath was of uniform concentration that a uniform coating could be obtained providing the current density was uniform.

I have found that when continuously electroplating strip, and especially at speeds of about 1,000 feet per minute or more, the strip drags along the solution that is in contact with its bottom surface at a speed greater than the rate of flow of the solution inwardly toward the middle of the strip. As a result, there is apparently a void or depression formed in the solution at a zone midway of the sides of the strip adjacent the entry end of the cell. The exact nature of what takes place in the solution below the middle of the bottom surface can not be visually observed but the answer which I have discovered to the problem indicates that this zone of reduced contact has been the difficulty. It has been found that if all of the electrolyte solution which is discharged into the cell below the level of the strip is discharged in the form of a single stream directed upwardly against the bottom surface at the middle of the strip width and adjacent the entry end of the cell, the void is filled and a more uniform coating is obtained and the middle portion of the surface has a coating of about the same thickness as the edge portions.

The present invention and its objects and advantages will become more readily apparent from the following detailed description, taken in connection with the accompanying drawings, in which:

Figure 1 is a plan view of a portion of an electroplating line including an electroplating cell embodying the principles of the present invention:

Figure 2 is a sectional view taken along line 2—2 of Figure 1;

Figure 3 is a transverse sectional view taken along line 3—3 of Figure 2 with some parts omitted for a better understanding of the present invention.

Referring more particularly to the apparatus shown in the accompanying drawings, a ferrous metal strip 10 is continuously moved from left to right along the electroplating line and passes from a preceding cell 11 between an upper contact roll 12 and a lower backup roll 13. The strip 10 then passes across the cell 14 and between an upper contact roll 15 and a lower backup roll 16 to a succeeding cell 18. The rotatable contact rolls 12 and 15 are connected to a source of electric current (not shown) and the backup rolls 13 and 16 are usually formed of rubber. The rolls may be power-driven but ordinarily, the strip 10 is continuously moved along the line by any one of the usual power-actuated roll means customarily used in mills for continuously moving strip along a path.

After the strip 10 leaves rolls 12 and 13, it passes across cell 14 from the entry end to the exit end and has a layer of protective tin deposited on its bottom surface. Cell 14 is similar to the other cells in the electroplating line and may be the first, last or intermediate one of a series of cells or may be the only cell for plating the bottom surface of the strip. Cell 14 includes a tray 19 supported by the framework 20 and containing an open, plating bath of electrolyte solution 11, Figure 3. The term "open" means that the upper surface of the bath is free so that the strip can drag solution from the entry end of the tray to the exit end of the tray. The cell tray 14 contains a tin anode formed of a plurality of tin anode elements or bars 21 each having one end supported on a conductive member 22. Spaced insulated members 23 are pro-

vided in tray 19 for supporting the other ends of the anode elements 21. Conductive member 22 is provided at one end with bus bars 25 adapted to be connected to the source of electricity to complete the electroplating circuit. The upper, anode-supporting surfaces of the conductive member 22 and insulated members 23 extend transversely of the direction of strip travel and these anode supporting surfaces are inclined so that the anode elements can be moved up these surfaces as they erode as a result of the electrodeposition of the anode metal on the bottom surface of strip 10. New anode elements are inserted at 27 (Figures 1 and 3) and eroded elements are removed at 28. Normally the anode elements are positioned so that the upper surfaces are located in a plane substantially parallel to the strip and so that the width of the anode is substantially the same as the width of the strip to produce a substantially uniform current density across the strip surface.

The tray includes a side wall 30 at the entry end which terminates slightly below the pass line of the strip. The level of the sidewall 30 controls the level of the bath in the tray for any one rate of flow of solution into the tray and at any one speed of strip travel. Solution is fed into the tray 19 as will be more fully hereinafter described. The top of sidewall 30 is such that the level of the surface of the bath of solution in the tray with the strip 10 stationary would be at or slightly above the level of the bottom surface of the strip as is indicated in Figure 3. The strip preferably should just touch the bath but to insure contact between the bath and the strip surface, the bath surface often is maintained slightly above this level. The rapidly moving strip 10 drags solution along toward the rolls 15 and 16 and means are provided to confine the solution dragged along by the strip and force the solution flowing out of the cell to flow across the top of sidewall 30 in a direction opposite the direction of strip travel. The walls at 31 and 32 at opposite sides of tray 19 extend upwardly above the strip far enough to prevent the flow of solution laterally over their tops. The exit end wall 33 is provided with a resilient member 34 which substantially fluid-tightly engages the lower roll 16. Extensions 35 are provided for walls 31 and 32 that extend forwardly to the rolls 15 and 16. The solution dragged along the upper surface of the strip cannot flow past the contact roll 15 and builds up in front of the roll. When this dragged solution builds up to a sufficient height, it flows rearwardly and across the top of wall 30. Trays 36 are provided between the adjacent portions of the cells to catch the solution flowing across wall 19 and to catch the relatively small amount of solution which leaks past the rolls and other elements at the exit side of the tray. This collected solution may be pumped back into the cells. Before pumping the solution into the cells, additions are made to the solution to maintain the proper concentration of salts in the bath.

Fresh solution is flowed into tray 19 to replenish the bath and to replace the solution flowing out of the tray. Heretofore, the replenishing solution has been added in a haphazard manner to the cell at a point or points either above or below the strip.

In the present apparatus a flanged tube 37 is fastened to the side 31 of tray 19 and is connected through nipple 38 to one leg of a T connection 39. A second, upper bent tube 40 is

connected to another leg of the T member 39 which is in turn connected through a pipe 41 to a source of electrolyte solution under pressure. A valve 41' is provided for controlling the rate of flow through tube 40. The outlet portion 42 of tube 37 terminates in a single outlet orifice at 43. The outlet portion 42 is bent upwardly and is so positioned that the stream issuing from the outlet orifice is directed upwardly against the bottom surface on a zone at the middle of the sides of the strip and adjacent the entry of the cell tray. The zone where the stream from outlet orifice 43 impinges is ahead of the anode so that this stream impinges against the strip surface before the surface passes across and above the anode. The moving strip apparently drags along the solution immediately adjacent the strip to form a void beneath the strip. This void may have the configuration indicated by the broken line 44 on Figure 3 depending on the rate of travel of the strip and other factors. When this void is present, there is a zone of no contact with the strip and the bath which results in a zone of reduced thickness of tin. The reduction in thickness of the tin along the middle portion of the bottom surface is a function of the rate of travel of the strip and is more pronounced at speeds of about 1,000 feet per minute or higher. Regardless of the exact nature of the cause of the decreased thickness of tin along the middle of the strip, it has been found that directing the electrolyte solution up against a zone midway of the strip and adjacent the entry end of the tray, reduces the difference between the thickness of the tin coating adjacent the edges and at the center and apparently fills this void. For example, samples were taken of continuously plated strip. Part of the plated strip was quarter-pound plate and the remainder was half-pound plate. A portion of the strip of each weight was plated in accordance with the present process in which all of the electrolyte solution added to the cell at a point below the strip was directed as a single stream upwardly against the bottom surface in a zone midway of the strip sides and adjacent the entry end of the cell. The remainder of the strip was plated under the same conditions except that the solution was added in a customary manner to the cell as shown in the Rieger et al. Patent No. 2,399,254. The following sets forth the results obtained in which the quantities are in pounds of tin per base box:

*Strip coated in accordance with present invention*

| Strip Coated in Accordance with Present Invention |        |      |        | Strip Coated in Customary Manner |        |      |        |
|---------------------------------------------------|--------|------|--------|----------------------------------|--------|------|--------|
| Edge                                              | Center | Edge | Spread | Edge                             | Center | Edge | Spread |
| QUARTER-POUND PLATE                               |        |      |        |                                  |        |      |        |
| .25                                               | .24    | .25  | .01    | .27                              | .20    | .27  | .07    |
| HALF-POUND PLATE                                  |        |      |        |                                  |        |      |        |
| .47                                               | .48    | .48  | .01    | .50                              | .40    | .50  | .10    |

The above figures show the great improvement in the uniformity of the thickness of the tin coating obtained with the present invention. This not only reduces the number of rejects but also reduces the cost in that it is not necessary to plate the edge portions excessively to obtain the desired thickness of coating at the center.

The stream of solution directed upwardly against the middle of the bottom surface should be under sufficient pressure to impinge against the bottom surface and spread over the middle portion. If the strip were not present, the stream should rise to a level above the strip and above the quiescent level of the bath. The velocity and rate of flow of this upwardly directed stream can be varied, at least to a certain extent, by means of valve 41'. The outlet orifice at 43 is circular, but especially when relatively wider strip is being plated, the outlet orifice may be widened so as to extend laterally a greater distance than the orifice extends in the direction of strip travel.

I claim:

1. In apparatus for progressively electroplating only the bottom surface of strip with protective metal while the strip is continuously moving along a path, said apparatus comprising an electroplating cell including open tray means adapted to confine an open bath of electroplating solution, said tray means having an upwardly extending wall at its entry end terminating below the path of the strip, sidewalls at opposite sides of the tray means extending above the path of the strip, and wall means at the exit end of the tray means extending above the path of the strip whereby substantially all of the solution circulating through the cell flows rearwardly across the top of the wall at the entry end of the cell in a direction countercurrently to the direction of strip travel; a soluble anode of protective metal in the tray means below the path of the strip; means connecting the anode and the strip to a source of electroplating current as anode and cathode, respectively; means for supporting and horizontally moving the strip forwardly along such path across the tray from the entry end to the exit end with the bottom of the surface in contact with the bath and above the anode at a speed of at least 1,000 feet per minute whereby only the bottom surface is electroplated with anode metal; and means for discharging electroplating solution into said tray and against said strip, said last mentioned means consisting of means including an outlet positioned above the path of the strip arranged to discharge electroplating solution onto the top surface of the strip and consisting of means extending into the tray below the path of the strip and having a single outlet orifice positioned below the path of the

strip between the anode and the wall at the entry end of the tray and arranged to discharge a single stream of electroplating solution upwardly against the bottom surface of the strip in a zone at the middle of the strip width adjacent the entry end of the tray and ahead of the anode.

75 2. In apparatus for progressively electroplat-

ing only the bottom surface of continuously moving strip with protective metal, said apparatus comprising an electroplating cell including tray means adapted to confine an open bath of electroplating solution, said tray means having an upwardly extending wall at its entry end terminating below the path of the strip, sidewalls and wall means at the exit end of the tray means all extending above the path of the strip whereby substantially all of the solution circulating through the cell flows rearwardly across the top of said entry end wall; a soluble anode of protective metal in the tray means below the path of the strip; means for connecting the anode and the strip to a source of electroplating current as anode and cathode, respectively; means for supporting and horizontally moving the strip forwardly along a path across the tray means from the entry end to the exit end with the bottom surface of the strip in contact with the bath in the tray and at such a speed that the electroplating solution below the strip is dragged along by the strip toward the exit end of the tray means in an amount sufficient to form a void in the bath beneath the middle portion of the bottom surface of the strip and the bath solution whereby the protective metal coating along the middle portion is of reduced thickness; and means for discharging electroplating solution into the tray at a point below the strip, said means consisting of a conduit terminating in a single outlet orifice positioned to discharge a stream of electroplating solution upwardly against the bottom surface of the strip in a zone at the middle of the strip width and adjacent the entry end of the tray and ahead of the anode to fill said void with solution whereby the thickness of the protective metal coating along the middle portion of the bottom surface is increased.

3. In apparatus for progressively electroplating only the bottom surface of continuously moving strip with protective metal, said apparatus comprising an electroplating cell including tray means adapted to confine an open bath of electroplating solution, said tray means having an upwardly extending wall at its entry end terminating below the path of the strip, sidewalls and wall means at the exit end of the tray means all extending above the path of the strip whereby substantially all of the solution circulating through the cell flows rearwardly across the top of said entry end wall; a soluble anode of protective metal in the tray means below the path of the strip; means for connecting the anode and the strip to a source of electroplating current as anode and cathode, respectively; means for supporting and horizontally moving the strip along a path across the tray means from the entry end to the exit end with the bottom of the surface in contact with the bath in the tray and at such a speed that the electroplating solution below the strip is dragged along by the strip toward the exit end of the tray means in an amount sufficient to form a void in the bath beneath the middle portion of the bottom surface of the strip and the bath solution whereby the protective metal coating along the middle portion is of reduced thickness; and means for discharging electroplating solution into said tray and against said strip, said last-mentioned means consisting of means including an outlet orifice positioned above the path of the strip arranged to discharge electroplating solution onto the top surface of the strip and consisting of means having a single outlet orifice positioned below the

path of the strip arranged to discharge a single stream of electroplating solution upwardly against the bottom surface of the strip in a zone at the middle of the strip width and adjacent the entry end of the tray and ahead of the anode.

4. In apparatus for progressively electroplating only the bottom surface of continuously moving strip, said apparatus comprising an electroplating cell including tray means adapted to confine an open bath of electroplating solution, said tray means having an upwardly extending wall at its entry end terminating below the path of the strip, sidewalls and wall means at the exit end of the tray means all extending above the path of the strip whereby substantially all of the solution circulating through the cell flows rearwardly across the top of said entry end wall; a soluble anode of protective metal in the tray below the path of the strip; means for connecting the anode and the strip to a source of electroplating current as anode and cathode, respectively; means for supporting and horizontally moving the strip along a path at a speed of at least 1,000 feet per minute across the tray means from the entry end to the exit end with the bottom of the surface in contact with the bath in the tray whereby electroplating solution below the strip is dragged by the strip from the entry end toward the exit end of the tray means in an amount sufficient to form a void in the solution below the middle of the bottom surface of the strip adjacent the entry end of the tray; and means for discharging electroplating solution into the tray at a point below the strip, said means consisting of a conduit means terminating in a single outlet orifice positioned to discharge a stream of electroplating solution upwardly against the bottom surface of the strip in a zone at the middle of the strip width and adjacent the entry end of the tray and ahead of the anode to fill said void with solution whereby the thickness of the protective metal coating along the middle portion of the bottom surface is increased.
5. In apparatus for progressively electroplating the bottom surface of continuously moving strip, said apparatus comprising an electroplating cell including tray means adapted to confine an open bath of electroplating solution, said tray means having an upwardly extending wall at its entry end terminating below the path of the strip, sidewalls and wall means at the exit end of the tray means all extending above the path of the strip whereby substantially all of the solution circulating through the cell flows rearwardly across the top of said entry end wall; a soluble anode of protective metal in the tray means below the path of the strip; means for connecting the anode and the strip to a source of electroplating current as anode and cathode, respectively; means for supporting and horizontally moving the strip along a path at a speed of at least 1,000 feet per minute across the tray means from the entry end to the exit end with the bottom of the surface in contact with the bath in the tray whereby electroplating solution below the strip is dragged by the strip from the entry end toward the exit end of the tray means in an amount sufficient to form a void in the solution below the middle of the bottom surface of the strip adjacent the entry end of the tray; and means for discharging electroplating solution into the tray and against said strip, said means consisting of means including an outlet orifice positioned

above the path of the strip, arranged to discharge electroplating solution onto the top surface of the strip and consisting of means having a single outlet orifice positioned below the path of the strip arranged to discharge a single stream of electroplating solution upwardly against the bottom surface in a zone at the middle of the strip width and adjacent the entry end of the tray and ahead of the anode to fill said void.

6. In apparatus for progressively electroplating only the bottom surface of continuously horizontally moving strip, said apparatus comprising an electroplating cell including a tray adapted to contain an open bath of electroplating solution, an anode of protective metal in the tray below the path of the strip, and means causing the solution to flow from the tray only at the entry end of the tray and only in a direction opposite to the direction of strip travel; means for connecting the anode and the strip to a source of electroplating current as anode and cathode, respectively; means for supporting and horizontally moving the strip at a speed of at least 1,000 feet per minute across the tray from the entry end to the exit end with the bottom surface of the strip in contact with the surface of the bath in the tray whereby the bottom surface is plated with anode metal and the electroplating solution below the strip is dragged in the direction of strip travel to tend to form a zone of reduced contact between the middle portion of the strip bottom surface and the bath solution adjacent the entry end of the tray; and means for discharging electroplating solution into said tray and against said strip, said means consisting of means including an outlet orifice positioned above the path of the strip, arranged to discharge electroplating solution onto the top surface of the strip and consisting of means having a single outlet orifice positioned below the path of the strip arranged to discharge a single stream of electroplating solution upwardly against the bottom surface in a zone at the middle of the strip width and adjacent the entry end of the tray and ahead of the anode to fill said void.

7. In the process of progressively and continuously electroplating the bottom surface of continuously moving strip with protective metal, the steps comprising supporting and horizontally moving the strip along a horizontal path across an electroplating cell containing an open bath of electrolyte solution and a soluble anode of protective metal with the strip bottom surface in contact with the surface of the bath and above the anode while the strip is connected as a cathode to a source of electroplating current and while electrolytically depositing protective metal coating only on the bottom surface; and discharging electrolyte solution against the strip in the form of two streams only, and directing one stream against the upper surface of the strip and directing the other stream upwardly against the bottom surface in a zone at the middle of the strip width and adjacent the entry end of the cell and ahead of the anode.

8. In apparatus for progressively electroplating, only the bottom surface of continuously moving strip with protective metal, said apparatus comprising an electroplating cell including tray means adapted to confine an open bath of electroplating solution, said tray means having an upwardly extending wall at its entry end terminating below the path of the strip, sidewalls and wall means at the exit end of the tray all

extending above the path of the strip whereby substantially all of the solution circulating through the cell flows rearwardly across the top of said entry end wall; a soluble anode of protective metal in the tray below the path of the strip; means for connecting the anode and the strip to a source of electroplating current as anode and cathode, respectively; means for supporting and horizontally moving the strip forwardly along a path across the tray from the entry end to the exit end with the bottom surface of the strip in contact with the bath in the tray so that only the bottom surface is plated with anode metal; and means for discharging electroplating solution into the tray below the path of the strip, said last mentioned means terminating in a single outlet orifice positioned adjacent the entry end of the tray and ahead of the anode and below the path of the strip and said outlet orifice being positioned to discharge a stream of electroplating solution upwardly against the bottom surface of the strip in a zone at the middle of the strip width and adjacent the entry end of the tray and ahead of the anode.

9. In apparatus for progressively electroplating only the bottom surface of continuously moving strip with protective metal, said apparatus comprising an electroplating cell including tray means adapted to confine an open bath of electroplating solution, said tray means having an upwardly extending wall at its entry end terminating below the path of the strip, sidewalls and wall means at the exit end of the tray means all extending above the path of the strip whereby substantially all of the solution circulating through the cell flows rearwardly across the top of said entry walls; a soluble anode of protective metal in the tray below the path of the strip; means for connecting the anode and the strip to a source of electroplating current as anode and cathode, respectively; means for supporting and horizontally moving the strip forwardly along a path across the tray from the entry end to the exit end with the bottom surface of the strip in contact with the bath in the tray so that only the bottom surface is plated with anode metal; and means for discharging electroplating solution into said tray and against said strip, said last mentioned means including an outlet orifice positioned above the path of the strip arranged to discharge electroplating solution onto the top surface of the strip and a single outlet orifice positioned below the path of the strip adjacent the entry end of the tray and ahead of the anode, the outlet orifice positioned below the path of the strip being positioned to discharge a single stream of electroplating solution upwardly against the bottom surface of the strip in a zone at the middle of the strip width and adjacent the entry end of the tray and ahead of the anode.

10. The process claimed in claim 7 in which the electroplating cell includes an upwardly extending wall at its entry end terminating below the path of the strip and which includes the step of flowing across the top of the entry end wall in direction opposite to the direction of strip movement substantially all of the electrolyte solution circulating through the cell.

11. In the process of progressively and continuously electroplating the bottom surface of continuously moving strip with protective metal, the steps comprising supporting and horizontally moving the strip along a horizontal path across an electroplating cell from entry end to exit end, the cell including a tray containing an open bath

## 11

of electroplating solution and a soluble anode of protective metal and having an upwardly extending wall at the entry end of the tray terminating below the path of the strip, the strip being moved across the cell with the strip bottom surface in contact with the surface of the bath and above the anode while the strip is connected as a cathode to the source of electroplating current and while electrolytically depositing a protective metal coating only on the bottom surface and while flowing electrolyte solution from the tray only across the top of the entry end wall in a direction opposite the direction of strip travel; and discharging electrolyte solution into the tray at a level below the path of strip travel and directing all of this electrolyte solution in the form of a single stream upwardly against the bottom surface in a zone at the middle of the strip width

5

## 12

and adjacent to the entry end of the tray and ahead of the anode.

HARRY J. READING.

## REFERENCES CITED

The following references are of record in the file of this patent:

## UNITED STATES PATENTS

| Number    | Name          | Date          |
|-----------|---------------|---------------|
| 2,271,736 | Hall          | Feb. 3, 1942  |
| 2,307,928 | Hogaboom      | Jan. 12, 1943 |
| 2,395,437 | Venable       | Feb. 26, 1946 |
| 2,399,254 | Rieger et al. | Apr. 30, 1946 |

## 15 FOREIGN PATENTS

| Number | Country       | Date    |
|--------|---------------|---------|
| 986    | Great Britain | of 1896 |